

Oct. 14, 1930.

F. E. DE VRIES

1,778,185

PRINTER'S BLANKET OR THE LIKE

Filed May 15, 1929

Fig. 1



Fig. 2



Fig. 3



Fig. 5



Fig. 7



Fig. 8



Fig. 9



Inventor:

Ferron E. De Vries,

By W. Bartlett Jones, Atty

## UNITED STATES PATENT OFFICE

FENNO E. DE VRIES, OF EVANSTON, ILLINOIS, ASSIGNOR, BY MESNE ASSIGNMENTS, TO  
VULCAN PROOFING COMPANY, INC., OF BROOKLYN, NEW YORK, A CORPORATION  
OF NEW YORK

## PRINTER'S BLANKET OR THE LIKE

Application filed May 15, 1929. Serial No. 363,298.

The present invention relates generally to printers' blankets, and has particular reference to that type of blanket which is used on the impression roll of printing presses.

5 Impression surfaces of printers' blankets are preferred with a coating thereon which is oil-proof and ink-proof, that is, which is non-adhesive to ink so that there is no off-setting effect therefrom. This is particularly noticeable in the second impression roll of a 10 rotary press such as those on which newspapers are printed. In this field the web of paper passes over a first impression roll and the outside of the web is printed from the first 15 type roll. It then passes while still wet with ink so that the inked side passes over a second impression roll in order that the blank side of the web may be printed. The second impression roll should resist and repel the wet 20 ink, so that it will not adhere and transfer to the paper on the next revolution. In addition, the blankets require certain degrees of 25 firmness and resiliency which are well known to the art, and many types of blankets are known which meet these requirements.

The present invention has reference particularly to the coating or impression surface, and provides a new material for the purpose, which may be used on any existing blanket, or 30 which may be used in new types of blankets permitted by the use of the new composition coating. Accordingly, the present invention is not to be considered as limited to the coating composition herein disclosed by way of 35 exemplifying the invention, but is to be considered in its broadest aspect as presented in the following description of the invention, and as expressed in the appended claims.

40 My invention depends upon the formation chemically in situ of a coating or surface-presenting composition in connection with printers' blankets and like materials. Broadly my invention comprises the application of 45 substances which are capable of reaction in situ to form a surface-presenting composition which has the desired properties. In practicing the invention I employ such substances as are capable of being applied or manipulated in a potentially reactive form, and which

can be reacted in situ to form a new product having the desired properties.

All material which is used in a blanket must have a flexibility sufficient to permit handling the blanket, to permit wrapping it around an impression cylinder, to permit bending it to 55 secure it to the cylinder, to form a suitable cushion during the period of impression. The coating must be tough, sufficiently hard, and durable, and as said above, it must be 60 oil proof and ink-repellent, when no other cover is employed. It is a custom in the art to use a draw sheet over a roll, when a coating on the blanket does not have all the 65 desirable properties. Therefore, in setting forth this invention I do not intend to limit it to the use of compositions which provide all the desirable properties, but I do claim that it permits and provides for the use of a material which is capable of imparting all 70 the above mentioned desirable properties to a printer's blanket, so that it may be used directly without additional means.

The primary object of the invention is the 75 use in forming a printer's blanket of a potentially reactive substance which is capable of reaction in situ to form a component part of the blanket.

Another object of the invention is the 80 use of such a substance in liquid or viscous form, which can be placed in the structure as a cement, as a coating, or as an impregnant, and there reacted to form a solid flexible product.

Still another object of the invention is the 85 provision of a coating composition which can be applied in potentially reactive form and which is reactive to form a solid flexible coating having all the properties above mentioned as desirable ones for printers' 90 blankets.

It is another object of the invention to employ compositions which upon reaction form 95 synthetic resins, and to modify the composition to modify the physical properties of the resin as desired.

It is a particular object of the invention to use a phenol-condensation product in direct or modified form which upon reaction 100

forms a flexible coating of the character desired.

It is a further object of the invention to provide a rubber faced blanket with a non-peeling, oil proof coating formed in situ.

Various other objects and advantages of the invention will appear from the following description of a number of printers' blankets and compositions therefore which are disclosed herein, having reference to the accompanying drawings.

It is well known that rubber is damaged by use as an impression surface in printers' blankets. To obviate this difficulty and to eliminate the use of a "draw-sheet" over rubber blankets, and also over cork and felt blankets, it has been the practice to provide the blanket itself with an oil-proof coating. Such coatings are known which are also ink-

20 repellent, such as oxidized vegetable oils applied to the blanket, and nitrocellulose films modified with an emollient such as castor oil. These compositions are usually applied as plastic masses which dry in place, 25 or from solutions in volatile solvents which evaporate and leave a residue. Such coatings are subject to peeling, are not entirely flexible and impervious to oils and ink solvents, and are gradually affected by the

30 solvent action of the ink and will crack when bent, permitting the ink to soak into the felt. Accordingly they break down after a period of use. They may first weaken in spots or

35 pin holes, permitting the oil of the ink to penetrate into the felt, cork or rubber base which is beneath the coating. For this reason it has been a practice to place a fabric face layer over the resilient base, so that after the coating has broken down the fabric face

40 layer may be peeled off and a new fabric face layer may be placed on the base. Such a protective face layer does not outlive the base. Because of the fact that the blanket is used or is usable for a period after a slight breakdown, the fabric face layer has been cemented to the cushion by an oil-proof cement which holds back oil that may leak through the broken down protective face layer.

The present invention in its preferred 50 aspect, as hereinafter described, permits the formation of a coating in situ which is totally insoluble and impenetrable, and which is not applied by evaporation from a solvent, which therefore permits dispensing with the 55 fabric face and the oil-proof cement above described, and which will have a long life so that it is not necessary to resurface the base, permitting economical replacement of the whole blanket when the life of the blanket is 60 exhausted.

As the preferred material for carrying out my invention in its preferred form, I employ a synthetic resin which is manufactured under the Byck Patent No. 1,590,079, which is 65 sold as "flexible bakelite" B. V. 1413 made by

the Bakelite Corp. of Delaware, and which is a potentially reactive phenol condensation product including in its composition an oil which is claimed to be chemically combined with the reactive resin-forming ingredients of the substance, which is capable of reaction, as by baking, to form a final reaction product having the characteristics of insolubility in organic solvents, oils and acids, which is water proof, and which is oil proof, and which I have discovered is also ink-repellent and non-offsetting in surface characteristics. It is flexible and in a thin coating is resilient, yet tough and hard to meet the purpose of a coating for printers' blankets. I have also 70 discovered that emollients, pigments, fillers, etc., may be incorporated into the reactive composition to be included within the final solid product to alter the physical characteristics in desired directions. I have also 75 learned that certain solvents may be employed for the reactive composition which alter the fluidity or viscosity of the mass which is utilized for applying it, and for incorporating modifying agents with it, and that the solvents cease to exert a solvent action when the substance is reacted into its final insoluble form.

I do not intend to limit myself to the use of the particular product of the Byck patent, 80 but aim to include other substances for forming synthetic resins, which may be dissolved and/or modified and then reacted in situ to form a new flexible composition. Substances such as the resins made by reacting glycerine and phthalic anhydride may be used as a base. However, the final reaction product of this class of resins is not insoluble in all solvents, and therefore I do not consider it preferred to the phenol-condensation resin 85 specified. Nor do I limit the invention to the use of the insoluble type of phenolic condensation product. It is well known that these resins may be formed with different degrees of solubility. For example, phenol and aldehydes may be condensed to form a resin. When the reactive phenolic constituent is in excess of the cooperating reactive 90 ingredient, a resin is formed which is soluble, and which has further capacity to react with more of the cooperative ingredient, until the final product is insoluble and infusible. The reacting substances may be present together and be un-reacted, and yet have a resin character. Such resins are capable of internal 95 change by reaction under heat to form a different resin, and when fully reacted are called finally reacted resins. The present invention aims to use products reacted in situ as the 100 composition which is new in the art, and preferably those which are finally reacted, and therefore stabilized. However, if further change toward stability does not materially 105 alter the product to render it non-effective 110

for its required purposes the question of stability need not be considered.

The resin-forming substance which I employ in the preferred form of my invention, preferably with suitable solvent and modifying agents may be used as a cement for securing fabric layers together, or for impregnating substances, such as textile fibers, or for coating materials or compositions, such as rubber faces, rubber impregnated fabrics, cork compositions or felt surfaces. The invention applies to bodies made wholly or partially of rubber, so that a rubber surface which, when in use, is exposed to the action of a substance injurious to rubber, must be protected against such substance. It will be noted that condensation products are generally referred to in the art as "resinous" products and these products are utilized for protecting the rubber surface. By providing a very viscous mass of the reacting substance, accomplished by control of the nature and amount of solvent, or by admixture of fillers such as aluminium stearate, the reactive mass may be applied to porous materials such as felt, or woolen or cotton fabric, in such a way as to minimize the impregnation of the fabric or material and to form a coating thereon which is attached to the substance without impregnating it deeply or appreciably. Non-porous substances, like a rubber surface may be coated with the composition by using a solvent which may penetrate or partially dissolve the rubber, thereby securing a non-peeling coating on the rubber, or other substance.

The reactive composition may be applied to materials in which a rubber compound is also present, and the product be subjected to heat to simultaneously effect vulcanization of the rubber and reaction of the composition to form a resin. Since rubber may be vulcanized at a temperature which is suitable for reacting the resin-forming substance, and since the resin-forming substance may be reacted at a temperature which will effect vulcanization, and since neither substance is destroyed during a suitable heat treatment of the other, various methods may be employed for using the resin substance and rubber in the same structure, with one heat treatment or with two or more heat treatments.

In the accompanying drawings there are shown a variety of combinations of structure that are suitable for printers' blankets using the composition herein described in various ways. In the drawings

Fig. 1 illustrates a rubber coated felt with an improved surface coating, to provide a printer's blanket.

Fig. 2 represents a felt body with a surface coating.

Fig. 3 represents a coating containing a filler in quantity to produce a rough coating.

Fig. 4 represents a coating having particles inlaid in the surface.

Fig. 5 represents a printer's blanket comprising a cushion or base fabric facing cemented thereto.

Fig. 6 represents the structure of Fig. 5 with an additional surface coating.

Fig. 7 represents a cushion with a composition coating having a fabric at the exposed surface thereof.

Fig. 8 represents the structure of Fig. 7 with an additional coating.

Fig. 9 illustrates a compound cushion material comprising resilient particles bonded with material which provides a suitable surface for a printer's blanket.

In order to explain the invention, I have chosen to illustrate it by describing how it may be carried out with a synthetic resin of the phenolic condensation type, and have chosen specifically the product known and identified in the trade as B. V. 1413, a form of "bakelite" above referred to. I have chosen this material as an illustration because it is obtainable on the market in a form suitable for use without modification, and also suitable for modification to vary and control the physical character of the resulting product. It is to be understood that other resins are available besides B. V. 1413 which are potentially reactive to form upon reaction a flexible coating, consequently I do not intend to be limited by this description to the specific material disclosed. It is also to be understood that those forms of resins which are not inherently flexible when reacted may be modified by incorporating in the unreacted mass a quantity of emollient, such as castor oil, neat's-foot oil, petroleum jelly, corn oil, and the like, and reacting the material to include the emollient. If the emollients are not soluble in the potentially reactive mass, a common solvent for the single or mixed emollients and the reactive substance may be employed, or the ingredients may be homogenized by emulsification. It is to be understood that in the exemplary disclosure, B. V. 1413 varnish is selected because it is readily available on the market, and is soluble in solvents to produce homogeneous mixtures with emollients, and particularly because it possesses the desirable properties for producing the coating directly without modification.

Another reason for selecting this material as a specific example is that it contains a solvent and is soluble in solvents containing benzol, which is also a solvent for rubber. This permits the material containing benzol or other rubber solvent to be applied to rubber, either before or after vulcanization to effect a perfect union of the resin to the rubber. It may be reacted by heat which may also vulcanize the rubber, and during the heat treatment it will not damage rubber which is already vulcanized or which

70

75

80

85

90

95

100

105

110

115

120

125

130

is unvulcanized, and it permits simultaneous vulcanization and resin formation.

I have coated the rubber surface of a rubberized felt with a varnish of the viscous B. V. 1413 substance as purchased on the market, spreading the same evenly by its natural flow. The coated sheet has been reacted in the usual manner, and I have found that heating for one hour at 145° C. effectively reacts the varnish, does not affect the rubber and does not injure the felt. The sheet is flexible, resilient, oil-proof and ink-repellent and has all the desirable properties of an impression blanket. The coating is very flexible, and does not crack with the greatest bending of the sheet to which it may be subjected, the test being much more severe than the conditions encountered in actual practice. The coating is tough and resists tension under which it is placed when the surface is bent backward. In Fig. 1, 10 indicates a felt body, 11 indicates a rubber layer spread or calendered thereon, and 12 indicates the resin coating.

The raw B. V. 1413 contains a solvent which evaporates on exposure causing the residue to thicken or get more viscous. Its power of penetration is thus decreased. The raw material may be permitted to lose solvent by evaporation so that where the base to be coated has a tendency to absorb, the absorption may be controlled by the amount and character of the solvent present. For example, in coating the fibrous surface of a felt body, I have found that penetration may be minimized by letting the solvent evaporate and then spreading the thickened coating on the felt with a knife blade. Baking for one hour at 145° C. is sufficient without damage to the felt. It is to be recognized that as the solvent in the varnish is decreased the coating has less tendency to spread or smooth out as it undergoes the heating treatment. The sample felt coated as above described may therefore present a rougher surface than when a more dilute varnish is employed. The surface character of the felt also tends to make it rougher. This is desirable as it effects a good frictional grip on paper passing over it in use. If it is desired to have a smooth coating, a second layer of varnish may be applied using more solvent than in the first, which solvent may be more or less than that contained in the raw commercial varnish. If desired metallic dust, such as bronze or aluminum powder may be incorporated in the second coating to give the final coat a metallic appearance. Aluminum makes it appear silver. The second coating may be baked for one hour at 145° C. without in any way injuring the first baked coating or the felt. In Fig. 2 13 represents a felt body covered with the first thickened layer of varnish and baked to form a layer indicated at 14. The dotted line 15 indicates the line of division between the first coat 14 and a second coat 16, and

the particles 17 indicate metal or other filler, such as aluminum powder.

It is not necessary to evaporate the solvent from the raw material to prevent penetration. I may add material to the raw varnish which will effect a thickening of the mass to be applied. For example, there may be an addition of aluminum stearate to thicken it, and the amount is to be determined by the result desired, as to penetration, and as to the character of surface which results. Just as the evaporated raw varnish may produce a rough surface, the addition of sufficient material, such as aluminum stearate, may effect the same result. However, it is to be noted that by adding the aluminum stearate, the base substance of the coating is diluted, and the properties may be somewhat different than in the article described with reference to the first coat of Fig. 2.

In coating rubber, it is desirable that the surface be well cleaned so that even adherence of the varnish is obtained. Sponging with any solvent, such as benzol, is a satisfactory way of cleaning the rubber surface. I have coated rubber surfaces, such as a rubber coated fabric, with a number of modified forms of the raw varnish, and in order to illustrate the character of change which may be effected by adding other materials, such as miscible emollients, a number of examples will be given. Both the quantity and the selection of individual or mixed addition agents should be considered, as the character of the product may be thus varied.

As emollients, I have used castor oil, neat's-foot oil and petroleum jelly. Castor oil gives the surface a tacky feel in the proportions in which I have used it. A certain degree of this may be desired in order to prevent slipping of paper over the surface. Neat's-foot oil appears to be the best. Petroleum jelly makes the surface feel oily.

Castor oil to the extent of 15% with 85% raw B. V. 1413 forms a tacky surface, and as the quantity of oil is decreased the tackiness also decreases. When the castor oil is increased to as high as 25% of the mixture the surface is extremely tacky and sticky.

Neat's-foot oil at a concentration of 15% in the mixture is very satisfactory. The product is not oily, tacky or sticky. The oil renders the coating softer and less polished than when the raw varnish alone is used. The coating retains its oilproof character and its non-off-setting properties. When 25% neat's-foot oil is used the desirable properties are retained, but the surface has an oily feel, but not so much so as to prevent the blanket from being used for the desired purpose.

Petroleum jelly at a concentration of 15% in the mixture is more oily than a corresponding proportion of neat's-foot oil.

Solid ingredients, such as the metal powder already mentioned, may be added for

certain purposes. For example in Fig. 3, the coating 18 has particles 19 which may impart to the surface a rough contour, shown in exaggerated form in the drawing. The 5 coating is shown covering all the particles, so that the surface is homogeneous in character. Frictional properties may be imparted to the coating by this method. The particles may be solid and unyielding, such as 10 the metal powder, and they may be yielding particles such as rubber or cork incorporated into the mix.

Fig. 4 shows a surface produced by sprinkling solid particles 21 such as metal powder, 15 or carborundum dust, on the unformed coating 20 either prior to or during baking so that the formed coating anchors them in place to provide a rough surface, which is non-homogeneous in character. Such a surface 20 may be off-setting or non-off-setting, depending to some extent upon the character of the surface provided by the imbedded material. If it is a metal surface it may be non-off-setting. In any event it is a friction surface, and will serve to hold to it any sheet 25 over it, such as a draw sheet or a passing web passing around a roll containing a blanket so surfaced.

The material which is applied in an unreacted form and then reacted in situ, as exemplified by the bakelite varnish above described and identified, is not limited to use in this art as a coating for the surface of blankets. As above stated it has penetrating qualities for absorptive material, and penetration may be increased by thinning the mass or varnish with a solvent. It may therefore be used to impregnate a fabric sheet which can be baked, to provide an oil-proof layer anywhere in a blanket structure. Such an impregnated sheet may be cemented to a cork base, a rubber base or a felt base, by any suitable cement, such as rubber cement. In Fig. 5 there is shown a resilient 45 body portion 22, such as a cushion of cork, rubber, or felt, as used in the art, onto which is cemented by cement 23, a fabric sheet 24, which may be thin muslin, previously impregnated and baked to form resin 25. The 50 muslin of the fabric layer, being protected by the impregnating resin, provides a resin surface of the desired properties, which surface may be rough and conform somewhat to the weave of the fabric employed. Fig. 55 6 shows the same structure as Fig. 5, having cushion 26, cement 27, impregnated fabric 28, and an additional quantity or coating of resin 29 thereon, which may be smoother, or rougher than that provided directly by the 60 impregnated fabric surface, with or without filler, as previously described. In Fig. 7 the structure of Fig. 5 is shown again with the distinction that the cement employed between the fabric 30 and the cushion 31, is also 65 resin that is baked in situ. Consequently,

the coating material 32 is adherent directly to the cushion and carries at its immediate surface the fabric 30. Such a blanket may be made in a variety of ways. For example, the cushion may be first coated with a resin 70 varnish and baked. The fabric may then be impregnated and while wet baked onto the coated cushion. Or the fabric may be first impregnated and baked, and the varnish be used as the cement to attach the impregnated fabric to the cushion. The fabric may be impregnated with the varnish, and the cushion coated with the varnish, the two placed 75 in contact and then baked.

Fig. 8 represents the product of Fig. 7 with 80 an additional layer of coating over the impregnated fabric surface. It may be described as a product comprising a cushion 33, and a coating 34 of resin, between the faces of which there is imbedded in the coating layer a fabric 35.

Blankets comprising comminuted cork and a binder are known to the art, and these are used without a coating. It is also known to prove with a nitrocellulose coating. The 90 composition of the present invention may be used with advantage as a coating for such composition directly, or with fabric or filler as previously described. The material may also be made to serve as a binder for the 95 cork particles, so that the surface which it presents has the desired surface characteristic without a distinct coating being applied. In Fig. 9 I show a blanket in which resin varnish is used as a binder for resilient particles, such as comminuted cork, or rubber. The mass is made so that the body of the product is essentially comprised of the 100 resilient particles, and the resin is merely the binder. A plastic mass is formed and is spread upon one or both sides of a sheet of sustaining fabric and baked, forming for example, the blanket having the sustaining fabric 36, the separated particles 37, and the binder and surface-forming resin 38.

The present invention provides for the construction of a variety of blankets in various modified forms, illustrating specifically a substance which is oil-proof and ink-repellent, which is tough, which may be smooth 115 and quite transparent, which may be easily colored by adding pigments or dyes, or metal powders, which is soluble in a preformed state in which it is used and applied, and which may be modified in such state to produce a variety of different properties or degrees of the same property. The invention therefore provides for compounding a material in a preformed state, which may be used as a surface varnish, as a cement, as an 120 impregnating agent, or as a bond, and which may then be reacted in situ, to form a flexible product having qualities desired in a printer's blanket.

A printer's blanket must be pliable in order 125

to enable it to be bent around the impression roller. It must likewise be stretchable because the blanket is tightly stretched around the impression roller. Hence, when the protective surface portion is applied directly to a rubber face, as shown in Fig. 1 herein, said protective surface portion must be pliable and it must also be stretchable to a certain extent. Otherwise, the protective layer would peel off leaving the rubber layer unprotected.

10 Hence, the invention is not to be restricted to printers' blankets, although it is particularly applicable for this purpose, but it also extends to other articles in which rubber must be protected against substances which tend to shorten the life of the rubber.

It will be noted that the rubber layer shown in Fig. 1 is necessarily soft and compressible.

15 The phrase "in situ" means that the protective material is transformed into its final state while it is in contact with the base to be protected. However, the invention, in its broader aspects, is not to be limited to the embodiment shown in Fig. 1, in which a pure condensation product is used as the surface layer of the article, and said surface layer is formed from a specific type of "bakelite" product. The invention covers an article in which the outer portion of the article includes 20 the protective material, and said outer portion need not necessarily form the directly exposed outer surface portion of the article, as shown in Fig. 4, for example.

I claim—

35 1. A printer's blanket comprising a base having an outer protective portion which includes a resinous phenol-condensation product, said condensation product being ink repellent.

40 2. As a new and useful article of manufacture, a body of pliable and stretchable rubber-surfaced material, said rubber surface being subjected to the influence of a substance injurious to the rubber when the article 45 is in use, said surface having a flexible protective layer which includes a resinous phenol-condensation product resistant to said first mentioned substance.

50 3. A method of protecting the rubber surface of a pliable and stretchable rubber-surfaced body against a substance injurious to the rubber, which consists in forming on said rubber surface a yieldable layer which includes a resinous condensation product which 55 can protect said surface against said substance, said product having been hardened and having been transformed into the protective condition by chemical reaction in situ.

4. A printer's blanket comprising a base 60 having an outer ink-repellent portion which includes a resinous substance, said resinous substance having been hardened and transformed into ink-repellent condition by chemical reaction in situ.

65 5. A printer's blanket comprising a base

having an outer ink-repellent portion which includes a resinous condensation product admixed with a substance adapted to increase the flexibility of said resinous product, said resinous product having been hardened and 70 transformed into ink-repellent condition by chemical reaction in situ.

6. As a new and useful article of manufacture, a body of pliable and stretchable rubber surfaced material, the rubber surface being subjected to the influence of a substance injurious to the rubber when the article is in use, said surface having a flexible layer which includes protective resinous material resistant to said substance, said protective resinous material having been hardened and having been transformed into the protective condition by chemical reaction in situ.

7. A method of protecting the rubber surface of a pliable and stretchable rubber-surfaced body against a substance injurious to the rubber, which consists in forming on said surface by means of a heat reaction, a yieldable resinous protective layer which is 90 transformed by said heat reaction into final and protective form.

In witness whereof, I have hereunto affixed by signature.

FENNO E. DE VRIES. 95

100

105

110

115

120

125

130